# EUROPEAN PATENT SPECIFICATION

(11) **EP 4 432 314 B1**
(45) Date of publication and mention of the grant of the patent: **14.01.2026**
(21) Application number: 22939837.5
(22) Date of filing: 04.11.2022
(51) Int. Cl.: H01F 1/057, H01F 41/02, C22C 38/16

(54) **NEODYMIUM-IRON-BORON MAGNET MATERIAL AND PREPARATION METHOD THEREFOR AND APPLICATION THEREOF**
NEODYM-EISEN-BOR-MAGNETMATERIAL UND HERSTELLUNGSVERFAHREN DAFÜR UND ANWENDUNG DAVON
MATÉRIAU D'AIMANT NÉODYME-FER-BORE, SON PROCÉDÉ DE PRÉPARATION ET APPLICATION ASSOCIÉE

(30) Priority: 29.04.2022 CN 202210476515
(43) Date of publication of application: 18.09.2024
(73) Proprietor: Fujian Golden Dragon Rare-earth Co., Ltd., Longyan, Fujian 366300 (CN)
(72) Inventor: MOU, Weiguo, Longyan, Fujian 366300 (CN); WANG, Chen, Longyan, Fujian 366300 (CN); HUANG, Zhigao, Longyan, Fujian 366300 (CN); FU, Gang, Longyan, Fujian 366300 (CN); XU, Deqin, Longyan, Fujian 366300 (CN)
(74) Representative: Ström & Gulliksson AB
(86) International application number: PCT/CN2022/129742
(87) International publication number: WO 2023/207020

(56) References cited:
- EP-A1- 3 441 988
- WO-A1-2021/169893
- WO-A1-2021/244314
- CN-A- 101 542 644
- CN-A- 104 674 115
- CN-A- 106 653 268
- CN-A- 107 275 025
- CN-A- 111 243 809
- CN-A- 114 284 018
- JP-A- 2014 150 119
- US-A1- 2021 313 099

## Description

### FIELD OF THE INVENTION

The invention specifically relates to a neodymium-iron-boron magnet material, a preparation method, and use thereof.

### BACKGROUND OF THE INVENTION

The neodymium-iron-boron permanent magnet materials with Nd₂Fe₁₄B as the main component have higher remanence, coercivity and maximum magnetic energy product. They have excellent comprehensive magnetic properties and are widely used in high-tech fields such as computers, communications, and national defense. Motors are the main application field of neodymium-iron-boron permanent magnets, and their application in hybrid electric vehicles (HEVs) is particularly eye-catching. The drive motor is the core component of new energy vehicles, so the neodymium-iron-boron magnet materials with higher coercivity used in the drive motor have broad application prospects. At the same time, the improvement of the performance of drive motors forces the improvement of the performance of the neodymium-iron-boron magnet materials with higher coercivity to meet the magnet performance requirements of manufacturers for drive motor.

CN114284018A provides a NdFeB magnet, which includes main-phase grains with R₂(Fe,M)₁₄B structure and a grain-boundary phase. By controlling element ratios, grain size and using specific preparation methods, it can achieve high Br and Hcj, and is applicable in motors, especially in new-energy vehicles and energy-saving appliances.

EP3441988A1 provides sintered R-T- B based permanent magnet. It has a specific crystal structure with two types of grain boundaries and triple junction area phases. By controlling alloy composition, it can achieve high coercivity and squareness, and is suitable for various applications like wind power generation and new energy vehicles.

US2021313099A1 provides a R-T- B based permanent magnet. It contains main phase grains and grain boundary multiple junctions. Some junctions have a ZrB₂ crystal and an R-Cu- rich phase. The surface layer of main phase grains has heavy rare-earth elements, aiming to achieve high coercivity.

WO2021244314A1 provides a neodymium-iron-boron magnet material, its raw material composition, preparation method and applications. By controlling element ratios and processes, it has good grain boundary continuity, high remanence, coercivity, and excellent high-temperature and corrosion resistance.

Adding a certain amount of heavy rare earth elements Tb and Dy to the sintered neodymium-iron-boron master alloy can effectively improve the coercivity of the magnet. However, Tb and Dy are strategic metals with limited reserves and high prices. In addition, while improving coercivity, the remanence and magnetic energy product are sacrificed. Therefore, how to improve the intrinsic coercivity without using heavy rare earths or using less heavy rare earths is of great significance for reducing the cost of neodymium-iron-boron magnet materials.

### SUMMARY OF THE INVENTION

The technical problem solved by the present invention is to overcome the defects that the existing technology relies on heavy rare earth elements to improve the coercivity of neodymium-iron-boron magnet materials, which results in higher cost, limited sources of raw materials, and reduced remanence and magnetic energy product. The invention provides a neodymium-iron-boron magnet material, a preparation method, and use thereof. The neodymium-iron-boron magnet material of the present invention can improve the intrinsic coercivity and reduce the cost without using heavy rare earth elements or using a small amount of heavy rare earth elements, while maintaining the performances of higher remanence, magnetic energy product and squareness.

The present invention solves the above technical problem through the following technical solutions:
The invention, as defined in claim 1, provides a neodymium-iron-boron magnet material, comprising a nanocrystalline Cu-rich phase located in an intergranular triangular zone, wherein: the nanocrystalline Cu-rich phase consists of elements TM, RE, Cu and Ga at an atom ratio of TM:RE:Cu:Ga=(1-20):(20-55):(25-70):(1-15); and a volume percentage of the nanocrystalline Cu-rich phase in the intergranular triangular zone is 4-12%, wherein TM comprises Fe and/or Co, and RE is a rare earth element.

In some preferred embodiments of the invention, the TM is Fe and/or Co.

In the nanocrystalline Cu-rich phase, the TM has an atom percentage of preferably 5-15%, more preferably 7%, 10%, 12%, 13%, 14% or 15%.
and/or, in the nanocrystalline Cu-rich phase, the RE has an atom percentage of preferably 25-55%, more preferably 26%, 32%, 34%, 38%, 39%, 44%, 50%.
and/or, in the nanocrystalline Cu-rich phase, the Cu has an atom percentage of preferably 30-60%, more preferably 35-55%, such as 45%, 58%, 52%, 33%, 42% or 31%.
and/or, in the nanocrystalline Cu-rich phase, the Ga has an atom percentage of 1-10%, preferably 2%, 4%, 7%, 9% or 10%.
or, the nanocrystalline Cu-rich phase consists of Fe₅₋₁₅RE₂₅₋₄₀Cu₄₅₋₆₀Ga₂₋₉, wherein numbers are atomic percentages of respective elements;
or, the nanocrystalline Cu-rich phase consists of Fe₁₀₋₁₅RE₃₀₋₅₀Cu₃₀₋₄₄Ga₇₋₁₀, wherein numbers are atomic percentages of respective elements;

In some preferred embodiments of the invention, the nanocrystalline Cu-rich phase consists of Fe₇RE₃₉Cu₄₅Ga₉, wherein numbers represent atomic percentages of respective elements.

In some preferred embodiments of the invention, the nanocrystalline Cu-rich phase consists of Fe₁₂RE₂₆Cu₅₈Ga₄, wherein numbers represent atomic percentages of respective elements.

In some preferred embodiments of the invention, the nanocrystalline Cu-rich phase consists of Fe₁₄RE₃₂Cu₅₂Ga₂, wherein numbers represent atomic percentages of respective elements.

In some preferred embodiments of the invention, the nanocrystalline Cu-rich phase consists of Fe₁₀RE₅₀Cu₃₃Ga₇, wherein numbers represent atomic percentages of respective elements.

In some preferred embodiments of the invention, the nanocrystalline Cu-rich phase consists of Fe₁₃RE₃₈Cu₄₂Ga₇, wherein numbers represent atomic percentages of respective elements.

In some preferred embodiments of the invention, the nanocrystalline Cu-rich phase consists of Fe₁₄RE₃₄Cu₄₂Ga₁₀, wherein numbers represent atomic percentages of respective elements.

In the invention, the volume percentage of the nanocrystalline Cu-rich phase in the intergranular triangular zone is preferably 4-9%, for example 4.5%, 4.2%, 6.1%, 6.6%, 7.5%, 7.8% or 8.5%.

Those skilled in the field know that the intergranular triangular zone refers to an intergranular phase formed between three crystal grains.

The invention further provides a neodymium-iron-boron magnet material, comprising the following components of Cu: 0.20-0.9wt%; and Ga: 0.02-0.35wt%, wherein contents of Cu and Ga satisfy 2≤Cu/Ga≤15, wherein the Cu and the Ga represent a mass percentage of Cu and Ga respectively, the percentages are mass percentages in the neodymium-iron-boron magnet material, and a total content of all components in the neodymium-iron-boron magnet material is 100%.

In the invention, the Cu has a content of preferably 0.25-0.8wt%, such as 0.25wt%, 0.35wt%, 0.50wt%, 0.60% or 0.75%.

In the invention, the Ga has a content of preferably 0.05-0.2wt%, such as 0.10wt%, 0.12wt%, 0.16wt% or 0.18wt%.

In the invention, the neodymium-iron-boron magnet material generally further comprises a rare earth element RE.

Wherein, the mass percentage of the RE in the neodymium-iron-boron magnet material can be conventional in the art, preferably 28-35wt%, such as 30wt%, 30.2wt%, 31wt%, 32wt% or 33wt%.

Wherein, the RE generally includes at least Nd, and preferably further includes Nd and Pr.

When the RE includes Nd and Pr, the content of Nd can be conventional in the art, preferably 23-32wt%, such as 23.25wt%, 24wt% or 24.75wt%.

When the RE includes Nd and Pr, the content of Pr can be conventional in the art, preferably 7-9wt%, such as 7.75wt%, 8wt% or 8.25wt%.

In some preferred embodiments of the invention, the RE preferably further comprises Dy.

Wherein, the Dy has a content of preferably 0.1-0.5wt%, more preferably 0.1-0.3wt%, for example 0.2wt%.

In the invention, the neodymium-iron-boron magnet material generally further includes Al.

Wherein, the Al content may be conventional in the art, preferably 0.05-2wt%, more preferably 0.1-1.5wt%, such as 0.3wt%, 0.5wt%, 0.8wt% or 1.0wt%.

In the present invention, the neodymium-iron-boron magnet material generally further includes B.

Wherein, the content of B can be conventional in the art, preferably 0.85-1.1wt%, such as 0.95wt%, 0.96wt% or 0.98wt%.

In the present invention, the neodymium-iron-boron magnet material generally further includes Fe.

Wherein, the content of Fe can be conventional in the art, preferably 60-70wt%, more preferably 62-69wt%, such as 63.7wt%, 65.01wt%, 65.66wt%, 67.17wt%, 67.27wt%, 67.07wt% or 67.32wt%.

In the present invention, the neodymium-iron-boron magnet material preferably further includes Co.

Wherein, the content of Co can be conventional in the art, preferably 0.1-3wt%, such as 0.5wt%, 0.8wt% or 1.0wt%.

In the present invention, the neodymium-iron-boron magnet material preferably further includes Zr.

Wherein, the content of Zr can be conventional in this field, preferably 0.05-1wt%, such as 0.1wt%.

In the present invention, the neodymium-iron-boron magnet material preferably further includes Ti.

Wherein, the content of Ti can be conventional in the art, preferably 0.05-1wt%, such as 0.1wt%.

In the present invention, the neodymium-iron-boron magnet material preferably further includes Nb.

Wherein, the content of Nb can be conventional in the art, preferably 0.1-0.3wt%, such as 0.15wt%, 0.18wt% or 0.20wt%.

In a preferable embodiment of the invention, the neodymium-iron-boron magnet material comprises the following components by mass% of Nd: 24.75%, Pr: 8.25%, Al: 1.00%, Cu: 0.25%, Ga: 0.12%, Co: 0.80%, Nb: 0.15%, B: 0.98% and Fe: 63.7%.

In a preferable embodiment of the invention, the neodymium-iron-boron magnet material comprises the following components by mass% of Nd: 24.00%, Pr: 8.00%, Al: 0.80%, Cu: 0.35%, Ga: 0.16%, Co: 0.50%, Zr: 0.10%, Ti: 0.10%, B: 0.98% and Fe: 65.01%.

In a preferable embodiment of the invention, the neodymium-iron-boron magnet material comprises the following components by mass% of Nd: 23.25%, Pr: 7.75%, Al: 0.50%, Cu: 0.50%, Ga: 0.18%, Co: 1.00%, Nb: 0.20%, B: 0.96% and Fe: 65.66%.

In a preferable embodiment of the invention, the neodymium-iron-boron magnet material comprises the following components by mass% of Nd: 30.00%, Dy: 0.20%, Al: 0.30%, Cu: 0.50%, Ga: 0.10%, Co: 0.50%, Nb: 0.18%, B: 0.95% and Fe: 67.27%.

In a preferable embodiment of the invention, the neodymium-iron-boron magnet material comprises the following components by mass% of Nd: 30.00%, Dy: 0.20%, Al: 0.30%, Cu: 0.60%, Ga: 0.10%, Co: 0.50%, Nb: 0.18%, B: 0.95% and Fe: 67.17%.

In a preferable embodiment of the invention, the neodymium-iron-boron magnet material comprises the following components by mass% of Nd: 30.00%, Dy: 0.20%, Al: 0.30%, Cu: 0.50%, Ga: 0.05%, Co: 0.50%, Nb: 0.18%, B: 0.95% and Fe: 67.32%.

In a preferable embodiment of the invention, the neodymium-iron-boron magnet material comprises the following components by mass% of Nd: 30.00%, Dy: 0.20%, Al: 0.30%, Cu: 0.75%, Ga: 0.05%, Co: 0.50%, Nb: 0.18%, B: 0.95% and Fe: 67.07%.

Those skilled in the field know that Nd is neodymium, Fe is iron, B is boron, Tb is terbium, Dy is dysprosium, Co is cobalt, Cu is copper, Ga is gallium, Al is aluminum, Mn is manganese, Zr is zirconium, Ti is titanium, and Nb is niobium.

The invention, as defined in claim 5, further provides a preparation method for a neodymium-iron-boron magnet material, comprising following steps of preparing a magnet blank from the respective components of the neodymium-iron-boron magnet material as described above; and subjecting the magnet blank to an aging treatment to achieve the neodymium-iron-boron magnet material, wherein the aging treatment comprises a primary aging and a secondary aging, and the secondary aging is performed at a temperature of 440-480°C.

In the present invention, the preparation method of the magnet blank can be conventional in the art. Generally, it can be achieved by subjecting the respective components for the neodymium-iron-boron magnet material to smelting, casting, pulverization, shaping and sintering in turn.

Wherein, the smelting temperature may be conventional in the art, preferably 1550°C or less, more preferably 1480-1550°C, such as 1520°C.

Wherein, the smelting is preferably carried out in a vacuum environment, and the absolute pressure of the vacuum environment is preferably 2×10⁻²Pa-8×10⁻²Pa, such as 5×10⁻²Pa.

Wherein, the casting method may be conventional in this field, preferably a rapid solidification casting method.

Wherein, the casting temperature may be conventional in the art, preferably 1390-1460°C, such as 1410°C.

Wherein, the thickness of the alloy casting sheet obtained after the casting can be conventional in this field, preferably 0.25-0.40 mm.

Wherein, the pulverization method can be conventional in this field, and preferably includes hydrogen decrepitation pulverization and jet mill pulverization in sequence.

The hydrogen decrepitation pulverization generally includes hydrogen absorption, dehydrogenation and cooling treatment.

In the hydrogen decrepitation pulverization, the hydrogen pressure during the hydrogen absorption process can be conventional in this field, preferably 0.05-0.12MPa, more preferably 0.085MPa.

In the hydrogen decrepitation pulverization, the dehydrogenation can be carried out by conventional methods in this field, preferably by raising the temperature under vacuum conditions. The temperature after heating can be conventional in the art, preferably 300-600°C, such as 500°C.

The atmosphere used for the jet mill pulverization can be conventional in this field, and preferably the oxidizing gas content is not higher than 100 ppm.

In the jet mill pulverization, the oxidizing gas can be conventional in the art and generally includes oxygen and/or water vapor.

The pressure in the grinding chamber during the jet mill pulverization can be conventional in this field, preferably 0.5-1MPa, more preferably 0.7MPa.

The particle size D50 after being pulverized by the jet mill pulverization can be conventional in this field, preferably 3-6 µm, such as 4.2 µm.

The particle size distribution after the jet mill pulverization can be conventional in this field, preferably D90/D10 is 3-5, more preferably 3.7.

Wherein, the shaping method can be conventional in this field, and is generally magnetic field molding.

The intensity of the magnetic field in the magnetic field shaping can be conventional in this field, and is preferably 1.8-2.5T.

Preferably, the magnetic field shaping is performed in a protective atmosphere. The protective atmosphere may be conventional in the art, such as nitrogen.

Wherein, preferably, a lubricant is added to the pulverized powder before the shaping.

Wherein, the lubricant can be conventional in this field, preferably zinc stearate.

The added amount of the lubricant can be conventional in the art, preferably 0.05-0.15%, more preferably 0.10%, wherein the percentage is the mass percentage of the lubricant and the pulverized powder.

Wherein, the sintering can be carried out using conventional methods in the art, preferably in a vacuum environment.

The vacuum condition can be conventional in the art, generally the absolute pressure is not higher than 10⁻²Pa, and more preferably is 5×10⁻³Pa.

Wherein, the sintering temperature may be conventional in the art, preferably 1000-1100°C, such as 1085°C.

Wherein, the sintering time can be conventional in the art, preferably 4-8 hours, such as 6 hours.

In the present invention, the primary aging can be carried out by conventional methods in this field, and generally heating is sufficient.

In the present invention, the temperature of the primary aging is preferably 800-1200°C, and more preferably 900°C.

In the present invention, the primary aging time is preferably 2-4 hours, more preferably 3 hours.

In the present invention, preferably, after the primary aging is completed, the material is cooled to room temperature and then the secondary aging is performed.

In the present invention, the temperature of the secondary aging treatment is preferably 440°C, 450°C, 460°C or 480°C.

In the present invention, the time of the secondary aging treatment is preferably 2-4 hours, more preferably 3 hours.

A neodymium-iron-boron magnet material is further prepared by the above preparation method.

The invention, as defined in claim 6, further provides use of the neodymium-iron-boron magnet material as described above as an electronic component in a motor.

In the present invention, the motor is preferably a new energy vehicle drive motor, an air conditioning compressor or an industrial servo motor, a wind turbine, an energy-saving elevator or a speaker assembly.

On the basis of common sense in the field, the above preferred conditions can be combined within the scope of the appended claims to obtain preferred examples of the present invention.

The reagents and raw materials used in the present invention are all commercially available.

The positive progressive effects of the present invention are as follows: In the case where the use of heavy rare earth elements is reduced or no heavy rare earth elements are added, the neodymium-iron-boron magnet material of the present invention still has significantly improved coercivity and remanence. The neodymium-iron-boron magnet material of the present invention has lower cost and broad prospects for large-scale production. As for the neodymium-iron-boron magnet material of the present invention, its remanence can be higher than 1.3T (13kGs), or even as high as 1.438T (14.38kGs), its intrinsic coercivity can be higher than 160.8 × 10⁴A/m (20.10kOe), or even as high as 209.6 × 10⁴A/m (26.20kOe); its maximum magnetic energy product can be higher than 320 × 10³J/m³ (40MGOe), even as high as 393.84×10³J/m³ (49.23 MGOe); and its squareness can be no less than 0.98, or even reach 0.99.

### BRIEF DESCRIPTION OF THE DRAWINGS

Fig. 1 shows the TEM pattern of the neodymium-iron-boron magnet material of Example 1;
Fig. 2 shows the TEM-EDS pattern of the neodymium-iron-boron magnet material of Example 1, wherein the arrow points to the nanocrystalline Cu-rich phase; and
Fig. 3 shows the high-resolution TEM pattern of the neodymium-iron-boron magnet material of Example 1.

### DETAILED DESCRIPTION OF THE INVENTION

The present invention is further described below by means of examples, but the present invention is not limited to the scope of the described examples. The experimental methods that do not indicate specific conditions in the following examples should be selected according to conventional methods and conditions, or according to product specifications.

### Examples 1-4 and Comparative Examples 1-5

The raw materials of respective Examples and Comparative Examples are prepared according to the composition list of the neodymium-iron-boron magnet materials shown in Table 1, and processed according to the following steps:
(1) Smelting: The prepared raw materials were put into a high-frequency vacuum induction melting furnace with a vacuum degree of 5×10⁻²Pa, and smelt into a molten liquid at a temperature of 1530°C.
(2) Casting: An alloy casting sheet with a thickness of 0.2-0.4mm was obtained by using the rapid solidification casting method at a casting temperature of 1420°C.
(3) Pulverization: The casting sheet obtained in step (2) was subjected to hydrogen decrepitation pulverization and jet mill pulverization in sequence.

The hydrogen decrepitation pulverization included hydrogen absorption, dehydrogenation and cooling treatment in sequence, in which the hydrogen absorption was carried out under the condition of hydrogen pressure of 0.085MPa. The dehydrogenation was carried out under the conditions of evacuation while heating, and the dehydrogenation temperature was 500°C.

The jet mill pulverization was carried out when the oxidizing gas (oxygen and moisture) content was 100ppm or less, and the pressure in the grinding chamber used for jet mill pulverization was 0.70MPa. The particle size D50 after pulverization was 4.1 µm, D90/D10 was 3.7, and a neodymium-iron-boron magnet material was obtained.
(4) Shaping: A lubricant zinc stearate was added into the neodymium-iron-boron magnet material in an amount of 0.10wt% of the neodymium-iron-boron magnet material, and then the neodymium-iron-boron magnet material was subjected to magnetic field shaping with a magnetic field strength of 1.8-2.5T under the protection of a nitrogen atmosphere.
(5) Sintering: The material was subjected to sintering under a vacuum condition of 5×10⁻³Pa and cooling. The sintering temperature was 1085°C. The sintering time was 6h. Before cooling, argon gas was introduced to bring the pressure to 0.05MPa.
(6) Aging treatment: The temperature of the primary aging was 900°C, and the time thereof was 3h, and then the treated material was cooled to room temperature. Then the temperature of the material was raised for the secondary aging. The temperatures for the secondary aging are shown in Table 2. The time of the secondary aging was 3h. A neodymium-iron-boron magnet material was obtained.

**Table 1 The list of the ingredients/% for the neodymium-iron-boron magnet materials in Examples and Comparative Examples**

| Examples/Comparative Examples | Nd | Pr | Dy | Al | Cu | Ga | Co | Zr | Nb | Ti | B | Fe |
|---|---|---|---|---|---|---|---|---|---|---|---|---|
| Example 1 | 24.75 | 8.25 | / | 1.00 | 0.25 | 0.12 | 0.80 | / | 0.15 | / | 0.98 | Balance |
| Example 2 | 24.00 | 8.00 | / | 0.80 | 0.35 | 0.16 | 0.50 | 0.1 0 | / | 0.1 0 | 0.98 | Balance |
| Example 3 | 23.25 | 7.75 | / | 0.50 | 0.50 | 0.18 | 1.00 | / | 0.20 | / | 0.96 | Balance |
| Example 4 | 30.00 | / | 0.20 | 0.30 | 0.50 | 0.10 | 0.50 | / | 0.18 | / | 0.95 | Balance |
| Example 5 | 30.00 | / | 0.20 | 0.30 | 0.60 | 0.10 | 0.50 | / | 0.18 | / | 0.95 | Balance |
| Example 6 | 30.00 | / | 0.20 | 0.30 | 0.50 | 0.05 | 0.50 | / | 0.18 | / | 0.95 | Balance |
| Example 7 | 30.00 | / | 0.20 | 0.30 | 0.75 | 0.05 | 0.50 | / | 0.18 | / | 0.95 | Balance |
| Comparative Example 1 | 24.75 | 8.25 | / | 1.00 | 0.25 | 0.20 | 0.80 | / | 0.15 | / | 0.98 | Balance |
| Comparative Example 2 | 24.75 | 8.25 | / | 1.00 | 1.00 | 0.3 | 0.80 | / | 0.15 | / | 0.98 | Balance |
| Comparative Example 3 | 24.75 | 8.25 | / | 1.00 | 0.15 | 0.06 | 0.80 | / | 0.15 | / | 0.98 | Balance |
| Comparative Example 4 | 24.75 | 8.25 | / | 1.00 | 0.25 | 0.12 | 0.80 | / | 0.15 | / | 0.98 | Balance |
| Comparative Example 5 | 24.75 | 8.25 | / | 1.00 | 0.25 | 0.12 | 0.80 | / | 0.15 | / | 0.98 | Balance |
| Comparative Example 6 | 30.00 | / | 0.20 | 0.30 | 0.75 | 0.60 | 0.50 | / | 0.18 | / | 0.95 | Balance |

| | | | | | | | | | | | | |
|---|---|---|---|---|---|---|---|---|---|---|---|---|
| Wherein, "/" means that the element was not added. The values of Fe content were obtained by subtracting the contents of other elements from 100%. Those skilled in the art know that the Fe content comprises some inevitable impurities introduced during the preparation process. | | | | | | | | | | | | |

### Effect Examples

### 1. Test of magnetic properties

By using the closed loop demagnetization curve testing equipment NIM-62000 manufactured by the China Institute of Metrology, the neodymium-iron-boron magnet materials obtained in Examples 1-4 and Comparative Examples 1-5 were tested at a testing temperature of 20°C to obtain the data on remanence (Br), intrinsic coercivity (Hcj), maximum magnetic energy product (BHmax) and squareness (Hk/Hcj). The testing results are shown in Table 2.

### 2. Characterization of microstructure

The neodymium-iron-boron magnet materials obtained in the Examples and Comparative Examples were tested by TEM. The SEM pattern of Example 1 is shown in Fig. 1. In Fig. 1, the triangular area marked by the dotted line is an intergranular triangular zone. Then, TEM-EDS element surface distribution scanning was used to find a Cu-rich area, as shown in the blue area in Fig. 2. The areas of the Cu-rich area and the intergranular triangular zone were calculated respectively. The area percentage of the nanocrystalline Cu-rich phase to the intergranular triangular zone was calculated and then converted into a volume ratio percentage. For the same material, its area percentage is the same as its volume percentage. The results are shown in Table 2.

Then, a high-resolution transmission electron microscopy was used to analyze the Cu-rich area. As shown in Fig. 3 (the neodymium-iron-boron magnet material obtained in Example 1), the textures with different orientations represent different crystal grains, and each unit with the same texture orientation represents a crystal grain in a Cu-rich area. It can be seen that the grain size is in a nanometer range.

### 3. Analysis of the components of the nanocrystalline Cu-rich phase

TEM-EDS (energy dispersion) analysis was used to quantitatively analyze the components of the nanocrystalline Cu-rich phases in respective Examples and Comparative Examples. The results are shown in Table 2 respectively.

**Table 2 Data for the ingredients of the neodymium-iron-boron magnet materials and the results of the magnetic properties**

| Example/ Comparative Example | Temperature for Secondary Aging /°C | Cu/Ga (Mass Ratio) | Volume Percentage of Nanocrystalline Cu-Rich Phase in Intergranular Triangular Zone /% | Composition of Nano-Cu-Rich Phase (Atomic Ratio /%) | Magnetic Properties | | | |
|---|---|---|---|---|---|---|---|---|
| | | | | | Bᵣ (T (kGs)) | H_{cJ} (A/m (kOe)) | BHmax (J/m³ (MGOe)) | Hₖ/H_{cJ} |
| Example 1 | 440 | 2.08 | 4.5 | Fe₇RE₃₉Cu₄₅Ga₉ | 1.301 (13.01) | 209.60×10⁴ (26.20) | 322.40×10³ (40.30) | 0.99 |
| Example 2 | 440 | 2.19 | 6.1 | Fe₁₂RE₂₆Cu₅₈Ga₄ | 1.343 (13.43) | 204.80×10⁴ (25.60) | 343.52×10³ (42.94) | 0.99 |
| Example 3 | 480 | 2.78 | 4.2 | Fe₁₄RE₃₂Cu₅₂Ga₂ | 1.397 (13.97) | 188.00×10⁴ (23.50) | 371.76×10³ (46.47) | 0.98 |
| Example 4 | 460 | 5 | 8.5 | Fe₁₀RE₅₀Cu₃₃Ga₇ | 1.438 (14.38) | 160.80×10⁴ (20.10) | 393.84×10³ (49.23) | 0.99 |
| Example 5 | 460 | 6 | 7.5 | Fe₁₃RE₃₈Cu₄₂Ga₇ | 1.437 (14.37) | 163.20×10⁴ (20.40) | 400.96×10³ (50.12) | 0.99 |
| Example 6 | 460 | 10 | 6.6 | Fe₁₄RE₃₄Cu₄₂Ga₁₀ | 1.438 (14.38) | 160.00×10⁴ (20.0) | 394.00×10³ (49.25) | 0.99 |
| Example 7 | 460 | 15 | 7.8 | Fe₁₅RE₄₄Cu₃₁Ga₁₀ | 1.433 (14.33) | 168.00×10⁴ (21.0) | 398.80×10³ (49.85) | 0.99 |
| Comparative Example 1 | 450 | 1.25 | None | / | 1.300 (13.00) | 200.00×10⁴ (25.00) | 321.92×10³ (40.24) | 0.94 |
| Comparative Example 2 | 450 | 3.5 | None | / | 1.295 (12.95) | 198.40×10⁴ (24.80) | 319.44×10³ (39.93) | 0.88 |
| Comparative Example 3 | 450 | 2.5 | 1.8 | Fe₁₂RE₄₂Cu₃₆Ga₁₀ | 1.299 (12.99) | 197.60×10⁴ (24.70) | 321.44×10³ (40.18) | 0.92 |
| Comparative Example 4 | 500 | 2.08 | None | / | 1.302 (13.02) | 196.80×10⁴ (24.60) | 322.88×10³ (40.36) | 0.94 |
| Comparative Example 5 | 430 | 2.08 | None | / | 1.300 (13.00) | 195.20×10⁴ (24.40) | 321.92×10³ (40.24) | 0.93 |
| Comparative Example 6 | 460 | 1.2 | None | / | 1.427 (14.27) | 148.80×10⁴ (18.60) | 395.20×10³ (49.40) | 0.89 |

In the ingredients of the nanocrystalline Cu-rich phase in Table 2, the numbers represent the atomic percentages of respective elements.

It can be seen from Table 2 that in the neodymium-iron-boron magnet materials produced by the present invention, a nanocrystalline Cu-rich phase having a specific area percentage was formed in the intergranular triangular zone. The inventor found through research that when the area percentage is 3-8%, the neodymium-iron-boron magnet materials have excellent magnetic properties. That is, when no heavy rare earth elements are added or less heavy rare earth elements are added and the remanence is higher than 1.3T (13kGs), or even as high as 1.438T (14.38kGs), the intrinsic coercivity is higher than 160 × 10⁴A/m(20kOe), or even as high as 209.6×10⁴A/m(26.20kOe). At the same time, its magnetic energy product and squareness performance are better. The magnetic energy product can be greater than 322.4×10³J/m³(40.30MGOe), or even as high as 393.84×10³J/m³ (49.23MGOe), and the squareness is higher than 0.98, or even as high as 0.99.

Comparative Example 1 does not meet the range of 2≤Cu/Ga≤6 defined in the present invention, which makes it impossible to form a nanocrystalline Cu-rich phase in the intergranular triangular zone of the neodymium-iron-boron magnet material, so that when the remanence is 1.3T (13kGs), the intrinsic coercivity is only 200×10⁴A/m (25kOe), which is not as good as the present invention. Comparative Example 2 indicates that when the Cu/Ga range of the present invention is met but the Cu content is too high, the nanocrystalline Cu-rich phase cannot be formed. Accordingly, the remanence and intrinsic coercivity of the obtained neodymium-iron-boron magnet material are significantly worse than those of the present invention, and the magnetic energy product and squareness are also worse than those of the present invention. Comparative Example 3 indicates that when the Cu/Ga range of the present invention is met but the Cu content is too low, although a nanocrystalline Cu-rich phase can be formed, the area percentage of the nanocrystalline Cu-rich phase is too small. Accordingly, the remanence and intrinsic coercivity of the obtained neodymium-iron-boron magnet material are significantly worse than those of the present invention, and the magnetic energy product and squareness are also worse than those of the present invention. Comparative Examples 4 and 5 indicate that when both of the Cu content and Cu/Ga meet the range defined by the present invention, if the temperature for the secondary aging is too high or too low, the nanocrystalline Cu-rich phase also cannot be formed. The magnetic properties such as remanence, intrinsic coercivity, magnetic energy product and squareness or the like of the corresponding neodymium-iron-boron magnet materials are all significantly worse than those of the present invention. Compared with Example 7, Comparative Example 6 only differs in Cu/Ga. The nanocrystalline Cu-rich phase cannot be formed in the obtained neodymium-iron-boron magnet material of Comparative Example 6. The remanence thereof is 1.4T (14kGs) or more but the intrinsic coercivity thereof is significantly worse than that of the present invention.

## Claims

1. A neodymium-iron-boron magnet material, **characterized in that**:
the neodymium-iron-boron magnet material comprises the following components by mass% of Nd: 23-25%, Pr: 7-9%, Al: 0.4-1.2%, Cu: 0.25-0.50%, Ga: 0.12-0.18%, Co: 0.70-1.50%, Zr: 0-0.2%; Nb: 0-0.20%, Ti: 0-0.1%, B: 0.96-0.98%; and a balance of Fe; or the neodymium-iron-boron magnet material comprises the following components by mass% of Nd: 28-32%, Dy: 0.1-0.3%, Al: 0.2-0.5%, Cu: 0.50-0.80%, Ga: 0.05- 0.10%, Co: 0.40-0.60%, Nb: 0.15-0.20%, B: 0.90-0.96% and a balance of Fe;
wherein contents of Cu and Ga satisfy 2≤Cu/Ga≤15, wherein the Cu and the Ga represent a mass percentage of Cu and Ga respectively, the percentages are mass percentages in the neodymium-iron-boron magnet material, and a total content of all components in the neodymium-iron-boron magnet material is 100%; and
wherein the neodymium-iron-boron magnet material comprises a nanocrystalline Cu-rich phase located in an intergranular triangular zone, wherein: the nanocrystalline Cu-rich phase consists of elements TM, RE, Cu and Ga at an atom ratio of TM:RE:Cu:Ga=(1-20):(20-55):(25-70):(1-15); and a volume percentage of the nanocrystalline Cu-rich phase in the intergranular triangular zone is 4-12%, wherein TM comprises Fe and/or Co, and RE is a rare earth element.

2. The neodymium-iron-boron magnet material according to claim 1, **characterized in that**:
the TM is Fe and/or Co; and/or
in the nanocrystalline Cu-rich phase, the TM has an atom percentage of 5-15%, preferably 7%, 10%, 12%, 13%, 14% or 15%; and/or
in the nanocrystalline Cu-rich phase, the RE has an atom percentage of 25-55%, preferably 26%, 32%, 34%, 38%, 39%, 44%, 50%; and/or
in the nanocrystalline Cu-rich phase, the Cu has an atom percentage of 30-60%, preferably 45%, 58%, 52%, 33%, 42% or 31%; and/or
in the nanocrystalline Cu-rich phase, the Ga has an atom percentage of 1-10%, preferably 2%, 4%, 7%, 9% or 10%; or
the nanocrystalline Cu-rich phase consists of Fe₅₋₁₅RE₂₅₋₄₀Cu₄₅₋₆₀Ga₂₋₉, wherein numbers are atomic percentages of respective elements; or
the nanocrystalline Cu-rich phase consists of Fe₁₀₋₁₅RE₃₀₋₅₀Cu₃₀₋₄₄Ga₇₋₁₀, wherein numbers are atomic percentages of respective elements; or
the nanocrystalline Cu-rich phase consists of Fe₇RE₃₉Cu₄₅Ga₉, Fe₁₂RE₂₆Cu₅₈Ga₄, Fe₁₄RE₃₂Cu₅₂Ga₂, Fe₁₀RE₅₀Cu₃₃Ga₇, Fe₁₃RE₃₈Cu₄₂Ga₇, Fe₁₄RE₃₄Cu₄₂Ga₁₀ or Fe₁₅RE₄₄Cu₃₁Ga₁₀, wherein numbers are atomic percentages of respective elements.

3. The neodymium-iron-boron magnet material according to claim 1, **characterized in that** the volume percentage of the nanocrystalline Cu-rich phase in the intergranular triangular zone is 4-9%, preferably 4.5%, 4.2%, 6.1%, 6.6%, 7.5%, 7.8% or 8.5%.

4. The neodymium-iron-boron magnet material according to claim 1, **characterized in that**:
the neodymium-iron-boron magnet material comprises the following components by mass% of Nd: 24.75%, Pr: 8.25%, Al: 1.00%, Cu: 0.25%, Ga: 0.12%, Co: 0.80%, Nb: 0.15%, B: 0.98% and Fe: 63.7%; or
the neodymium-iron-boron magnet material comprises the following components by mass% of Nd: 24.00%, Pr: 8.00%, Al: 0.80%, Cu: 0.35%, Ga: 0.16%, Co: 0.50%, Zr: 0.10%, Ti: 0.10%, B: 0.98% and Fe: 65.01%; or
the neodymium-iron-boron magnet material comprises the following components by mass% of Nd: 23.25%, Pr: 7.75%, Al: 0.50%, Cu: 0.50%, Ga: 0.18%, Co: 1.00%, Nb: 0.20%, B: 0.96% and Fe: 65.66%; or
the neodymium-iron-boron magnet material comprises the following components by mass% of Nd: 30.00%, Dy: 0.20%, Al: 0.30%, Cu: 0.50%, Ga: 0.10%, Co: 0.50%, Nb: 0.18%, B: 0.95% and Fe: 67.27%; or
the neodymium-iron-boron magnet material comprises the following components by mass% of Nd: 30.00%, Dy: 0.20%, Al: 0.30%, Cu: 0.60%, Ga: 0.10%, Co: 0.50%, Nb: 0.18%, B: 0.95% and Fe: 67.17%; or
the neodymium-iron-boron magnet material comprises the following components by mass% of Nd: 30.00%, Dy: 0.20%, Al: 0.30%, Cu: 0.50%, Ga: 0.05%, Co: 0.50%, Nb: 0.18%, B: 0.95% and Fe: 67.32%; or
the neodymium-iron-boron magnet material comprises the following components by mass% of Nd: 30.00%, Dy: 0.20%, Al: 0.30%, Cu: 0.75%, Ga: 0.05%, Co: 0.50%, Nb: 0.18%, B: 0.95% and Fe: 67.07%.

5. A preparation method for a neodymium-iron-boron magnet material **characterized by** comprising following steps of preparing a magnet blank from the respective components of the neodymium-iron-boron magnet material according to any one of claims 1-4; and subjecting the magnet blank to an aging treatment to achieve the neodymium-iron-boron magnet material, wherein the aging treatment comprises a primary aging and a secondary aging, and the secondary aging is performed at a temperature of 440-480°C;
wherein the primary aging is performed at a temperature of preferably 800-1200°C, more preferably 900°C;
the primary aging is performed for a time of 2-4h, more preferably 3h;
preferably, when the primary aging is completed, the magnet blank is cooled to room temperature and then subjected to the secondary aging;
the secondary aging treatment is performed at a temperature of preferably 440°C, 450°C, 460°C or 480°C;
the secondary aging treatment is performed for a time of preferably 2-4h, more preferably 3h;
the preparation method for the magnet blank preferably comprises subjecting the respective components for the neodymium-iron-boron magnet material to smelting, casting, pulverization, shaping and sintering in turn;
the smelting is performed at a temperature of preferably 1550°C or less, more preferably 1480-1550°C, and further preferably 1520°C;
the smelting is preferably carried out in a vacuum environment;
the smelting is preferably carried out according to a rapid solidification casting method;
the smelting is performed at a temperature of preferably 1390-1460°C, more preferably 1410°C;
the pulverization preferably comprises hydrogen decrepitation pulverization and jet mill pulverization in turn; the hydrogen decrepitation pulverization preferably comprises hydrogen absorption, dehydrogenation and cooling treatments; the hydrogen absorption is performed at a hydrogen pressure of preferably 0.05-0.12MPa, more preferably 0.085MPa; the dehydrogenation preferably comprises heating to 300-600°C under a vacuum condition; the jet mill pulverization is preferably carried out in an atmosphere with an oxidizing gas content of no more than 100 ppm; the jet mill pulverization is performed in a grinding chamber having a pressure of preferably 0.5-1MPa, more preferably 0.7MPa; the magnet blank obtained after the jet mill pulverization has a particle size D50 of preferably 3-6 µm, more preferably 4.2 µm;
the shaping is preferably magnetic field shaping; the magnetic field shaping is preferably carried out under a magnetic field intensity of 1.8-2.5T; the magnetic field shaping is preferably carried out in a protective atmosphere;
it is preferable to add a lubricant to a powder obtained after the pulverization before the shaping; the lubricant is preferably zinc stearate; the lubricant has a mass percentage of preferably 0.05-0.15%, more preferably 0.10% in the powder obtained after the pulverization; the sintering is preferably carried out in a vacuum environment; the sintering is performed at a temperature of preferably 1000-1100°C, more preferably 1085°C; and the sintering is performed for a time of preferably 4-8 hours, more preferably 6 hours.

6. Use of the neodymium-iron-boron magnet material according to any one of claims 1-4 as an electronic component in a motor.

## Patentansprüche

1. Neodym-Eisen-Bor-Magnetmaterial, **dadurch gekennzeichnet, dass** das Neodym-Eisen-Bor-Magnetmaterial die folgenden Komponenten in Massenprozent aufweist: Nd: 23-25 %, Pr: 7-9 %, Al: 0,4-1,2 %, Cu: 0,25-0,50 %, Ga: 0,12-0,18 %, Co: 0,70-1,50 %, Zr: 0-0,2 %; Nb: 0-0,20 %, Ti: 0-0,1 %, B: 0,96-0,98 % und der Rest Fe; oder das Neodym-Eisen-Bor-Magnetmaterial weist die folgenden Komponenten in Massenprozent auf: Nd: 28-32 %, Dy: 0,1-0,3 %, Al: 0,2-0,5 %, Cu: 0,50-0,80 %, Ga: 0,05-0,10 %, Co: 0,40-0,60 %, Nb: 0,15-0,20 %, B: 0,90-0,96 % und der Rest Fe;
wobei die Gehalte an Cu und Ga die Bedingung 2 ≤ Cu/Ga ≤ 15 erfüllen, wobei Cu und Ga jeweils den Massenanteil von Cu und Ga darstellen, die Prozentsätze Massenanteile im Neodym-Eisen-Bor-Magnetmaterial sind und der Gesamtgehalt aller Komponenten im Neodym-Eisen-Bor-Magnetmaterial 100 % beträgt; und
wobei das Neodym-Eisen-Bor-Magnetmaterial eine nanokristalline Cu-reiche Phase aufweist, die sich in einer intergranularen Dreieckszone befindet, wobei: die nanokristalline Cu-reiche Phase aus den Elementen TM, RE, Cu und Ga in einem Atomverhältnis von TM:RE:Cu:Ga=(1-20):(20-55): (25-70):(1-15) besteht; und der Volumenanteil der nanokristallinen Cu-reichen Phase in der intergranularen Dreieckszone 4-12 % beträgt, wobei TM Fe und/oder Co aufweist und RE ein Seltenerdelement ist.

2. Neodym-Eisen-Bor-Magnetmaterial nach Anspruch 1, **dadurch gekennzeichnet, dass**:
TM Fe und/oder Co ist; und/oder
in der nanokristallinen Cu-reichen Phase TM einen Atomprozentanteil von 5-15 %, vorzugsweise 7 %, 10 %, 12 %, 13 %, 14 % oder 15 % aufweist; und/oder
in der nanokristallinen Cu-reichen Phase das RE einen Atomprozentanteil von 25-55 %, vorzugsweise 26 %, 32 %, 34 %, 38 %, 39 %, 44 %, 50 % aufweist; und/oder
in der nanokristallinen Cu-reichen Phase das Cu einen Atomprozentanteil von 30-60 %, vorzugsweise 45 %, 58 %, 52 %, 33 %, 42 % oder 31 % aufweist; und/oder
in der nanokristallinen Cu-reichen Phase das Ga einen Atomprozentanteil von 1-10 %, vorzugsweise 2 %, 4 %, 7 %, 9 % oder 10 % aufweist; oder
die nanokristalline Cu-reiche Phase aus Fe₅₋₁₅RE₂₅₋₄₀Cu₄₅₋₆₀Ga₂₋₉ besteht, wobei die Zahlen die Atomprozentanteile der jeweiligen Elemente sind; oder
die nanokristalline Cu-reiche Phase aus Fe₁₀₋₁₅RE₃₀₋₅₀Cu₃₀₋₄₄Ga₇₋₁₀ besteht, wobei die Zahlen die Atomprozentanteile der jeweiligen Elemente sind; oder
die nanokristalline Cu-reiche Phase aus Fe₇RE₃₉Cu₄₅Ga₉, Fe₁₂RE₂₆Cu₅₈Ga₄, Fe₁₄RE₃₂Cu₅₂Ga₂, FeioRE₅oCu₃₃Ga₇, Fe₁₃RE₃₈Cu₄₂Ga₇, Fe₁₄RE₃₄Cu₄₂Ga₁₀ oder Fe₁₅RE₄₄Cu₃₁Ga₁₀ besteht, wobei die Zahlen die Atomprozentanteile der jeweiligen Elemente bezeichnen.

3. Neodym-Eisen-Bor-Magnetmaterial nach Anspruch 1, **dadurch gekennzeichnet, dass** der Volumenanteil der nanokristallinen Cu-reichen Phase in der intergranularen Dreieckszone 4 bis 9 %, vorzugsweise 4,5 %, 4,2 %, 6,1 %, 6,6 %, 7,5 %, 7,8 % oder 8,5 % beträgt.

4. Neodym-Eisen-Bor-Magnetmaterial nach Anspruch 1, **dadurch gekennzeichnet, dass**:
das Neodym-Eisen-Bor-Magnetmaterial die folgenden Komponenten in Massenprozent aufweist: Nd: 24,75 %, Pr: 8,25 %, Al: 1,00 %, Cu: 0,25 %, Ga: 0,12 %, Co: 0,80 %, Nb: 0,15 %, B: 0,98 % und Fe: 63,7 %; oder
das Neodym-Eisen-Bor-Magnetmaterial die folgenden Komponenten in Massenprozent aufweist: Nd: 24,00 %, Pr: 8,00 %, Al: 0,80 %, Cu: 0,35 %, Ga: 0,16 %, Co: 0,50 %, Zr: 0,10 %, Ti: 0,10 %, B: 0,98 % und Fe: 65,01 %; oder
das Neodym-Eisen-Bor-Magnetmaterial die folgenden Komponenten in Massenprozent aufweist: Nd: 23,25 % Pr: 7,75 %, Al: 0,50 %, Cu: 0,50 %, Ga: 0,18 %, Co: 1,00 %, Nb: 0,20 %, B: 0,96 % und Fe: 65,66 %; oder
das Neodym-Eisen-Bor-Magnetmaterial die folgenden Komponenten in Massenprozent aufweist: Nd: 30,00 %, Dy: 0,20 %, Al: 0,30 %, Cu: 0,50 %, Ga: 0,10 %, Co: 0,50 %, Nb: 0,18 %, B: 0,95 % und Fe: 67,27 %; oder
das Neodym-Eisen-Bor-Magnetmaterial die folgenden Komponenten in Massenprozent aufweist: Nd: 30,00 %, Dy: 0,20 %, Al: 0,30 %, Cu: 0,60 %, Ga: 0,10 %, Co: 0,50 %, Nb: 0,18 %, B: 0,95 % und Fe: 67,17 %; oder
das Neodym-Eisen-Bor-Magnetmaterial die folgenden Komponenten in Massenprozent aufweist: Nd: 30,00 %, Dy: 0,20 %, Al: 0,30 %, Cu: 0,50 %, Ga: 0,05 %, Co: 0,50 %, Nb: 0,18 %, B: 0,95 % und Fe: 67,32 %; oder
das Neodym-Eisen-Bor-Magnetmaterial die folgenden Komponenten in Massenprozent aufweist: Nd: 30,00 %, Dy: 0,20 %, Al: 0,30 %, Cu: 0,75 %, Ga: 0,05 %, Co: 0,50 %, Nb: 0,18 %, 5 B: 0,95 % und Fe: 67,07 %.

5. Verfahren zur Herstellung eines Neodym-Eisen-Bor-Magnetmaterials, **gekennzeichnet dadurch, dass** es folgende Schritte aufweist: Herstellen eines Magnetrohlings aus den jeweiligen Komponenten des Neodym-Eisen-Bor-Magnetmaterials nach einem der Ansprüche 1 bis 4; und Unterziehen des Magnetrohlings einer Alterungsbehandlung, um das Neodym-Eisen-Bor-Magnetmaterial zu erhalten, wobei die Alterungsbehandlung eine primäre Alterung und eine sekundäre Alterung umfasst und die sekundäre Alterung bei einer Temperatur von 440 bis 480°C durchgeführt wird;
wobei die primäre Alterung bei einer Temperatur von vorzugsweise 800 bis 1200°C, bevorzugter 900°C, durchgeführt wird;
die primäre Alterung für eine Zeit von 2 bis 4 Stunden, bevorzugter 3 Stunden, durchgeführt wird;
vorzugsweise der Magnetrohling nach Abschluss der primären Alterung auf Raumtemperatur abgekühlt und dann der sekundären Alterung unterzogen wird;
die sekundäre Alterungsbehandlung bei einer Temperatur von vorzugsweise 440°C, 450°C, 460°C oder 480°C durchgeführt wird;
die sekundäre Alterungsbehandlung für eine Zeit von 2 bis 4 Stunden, bevorzugter 3 Stunden, durchgeführt wird;
das Herstellungsverfahren für den Magnetrohling vorzugsweise das Schmelzen, Gießen, Pulverisieren, Formen und Sintern der jeweiligen Komponenten für das Neodym-Eisen-Bor-Magnetmaterial in dieser Reihenfolge aufweist;
das Schmelzen bei einer Temperatur von vorzugsweise 1550°C oder weniger, bevorzugter 1480 bis 1550°C und noch bevorzugter 1520°C, durchgeführt wird;
das Schmelzen vorzugsweise in einer Vakuumumgebung durchgeführt wird;
das Schmelzen vorzugsweise nach einem Schnellverfestigungs-Gießverfahren durchgeführt wird;
das Schmelzen bei einer Temperatur von vorzugsweise 1390 bis 1460°C, bevorzugter 30 bis 1410°C, durchgeführt wird;
die Pulverisierung vorzugsweise eine Wasserstoff-Dekrepitation-Pulverisierung und eine Strahlmühlen-Pulverisierung nacheinander auf weist; die Wasserstoff-Dekrepitation-Pulverisierung vorzugsweise eine Wasserstoffabsorption, eine Dehydrierung und eine Kühlung aufweist; die Wasserstoffabsorption bei einem Wasserstoffdruck von vorzugsweise 0,05 bis 0,12 MPa, bevorzugter bei0,085 MPa, durchgeführt wird; die Dehydrierung vorzugsweise das Erhitzen auf 300-600°C unter Vakuumbedingungen aufweist; die Strahlmühlenpulverisierung vorzugsweise in einer Atmosphäre mit einem Oxidationsgasgehalt von nicht mehr als 100 ppm durchgeführt wird; die Strahlmühlenpulverisierung in einer Mahlkammer mit einem Druck von vorzugsweise 0,5 bis 1 MPa, bevorzugter 0,7 MPa, durchgeführt wird; der nach der Strahlmühlenpulverisierung erhaltene Magnetrohling eine Partikelgröße D50 von vorzugsweise 3 bis 6 µm, bevorzugter 4,2 µm, aufweist;
die Formgebung vorzugsweise durch Magnetfeldformgebung erfolgt; die Magnetfeldformgebung vorzugsweise unter einer Magnetfeldstärke von 1,8 bis 2,5 T durchgeführt wird; die Magnetfeldformgebung vorzugsweise in einer Schutzatmosphäre durchgeführt wird;
wobei es bevorzugt ist, dem nach der Pulverisierung erhaltenen Pulver vor der Formgebung ein Schmiermittel zuzusetzen; das Schmiermittel vorzugsweise Zinkstearat ist; das Schmiermittel einen Massenanteil von vorzugsweise 0,05 bis 0,15 % aufweist, bevorzugter 0,10 % in dem nach der Pulverisierung erhaltenen Pulver; das Sintern vorzugsweise in einer Vakuumumgebung durchgeführt wird; das Sintern bei einer Temperatur von vorzugsweise 1000-1100°C, bevorzugter 1085°C, durchgeführt wird; und das Sintern für eine Zeit von vorzugsweise 4-8 Stunden, bevorzugter 6 Stunden, durchgeführt wird.

6. Verwendung des Neodym-Eisen-Bor-Magnetmaterials nach einem der Ansprüche 1-4 als elektronisches Bauteil in einem Motor.

## Revendications

1. Matériau d'aimant néodyme-fer-bore, **caractérisé en ce que** :
le matériau d'aimant néodyme-fer-bore comprend les constituants suivants en % en masse de Nd : 23 à 25 %, Pr : 7 à 9 %, Al : 0,4 à 1,2 %, Cu : 0,25 à 0,50 %, Ga : 0,12 à 0,18 %, Co : 0,70 à 1,50 %, Zr : 0 à 0,2 % ; Nb : 0 à 0,20 %, Ti : 0 à 0,1 %, B : 0,96 à 0,98 % ; et le reste de Fe ; ou le matériau d'aimant néodyme-fer-bore comprend les constituants suivants en % en masse de Nd : 28 à 32 %, Dy : 0,1 à 0,3 %, Al : 0,2 à 0,5 %, Cu : 0,50 à 0,80 %, Ga : 0,05 à 0,10 %, Co : 0,40 à 0,60 %, Nb : 0,15 à 0,20 %, B : 0,90 à 0,96 % et le reste de Fe ;
dans lequel les teneurs en Cu et Ga satisfont 2 ≤ Cu/Ga ≤ 15, dans lequel le Cu et le Ga représentent un pourcentage en masse de Cu et de Ga respectivement, les pourcentages sont des pourcentages en masse dans le matériau d'aimant néodyme-fer-bore, et une teneur totale de tous les constituants dans le matériau d'aimant néodyme-fer-bore est de 100 % ; et
dans lequel le matériau d'aimant néodyme-fer-bore comprend une phase nanocristalline riche en Cu située dans une zone triangulaire intergranulaire, dans lequel : la phase nanocristalline riche en Cu est constituée d'éléments TM, RE, Cu et Ga à un rapport atomique de TM:RE:Cu:Ga = (1 à 20) : (20 à 55) : (25 à 70) : (1 à 15) ; et un pourcentage en volume de la phase nanocristalline riche en Cu dans la zone triangulaire intergranulaire est de 4 à 12 %, dans lequel TM comprend Fe et/ou Co, et RE est un élément des terres rares.

2. Matériau d'aimant néodyme-fer-bore selon la revendication 1, **caractérisé en ce que** :
le TM est Fe et/ou Co ; et/ou
dans la phase nanocristalline riche en Cu, le TM possède un pourcentage atomique de 5 à 15 %, de préférence de 7 %, 10 %, 12 %, 13 %, 14 % ou 15 % ; et/ou
dans la phase nanocristalline riche en Cu, le RE possède un pourcentage atomique de 25 à 55 %, de préférence de 26 %, 32 %, 34 %, 38 %, 39 %, 44 % ou 50 % ; et/ou
dans la phase nanocristalline riche en Cu, le Cu possède un pourcentage atomique de 30 à 60 %, de préférence de 45 %, 58 %, 52 %, 33 %, 42 % ou 31 % ; et/ou
dans la phase nanocristalline riche en Cu, le Ga possède un pourcentage atomique de 1 à 10 %, de préférence de 2 %, 4 %, 7 %, 9 % ou 10 % ; ou
la phase nanocristalline riche en Cu est constituée de Fe₅₋₁₅RE₂₅₋₄₀Cu₄₅₋₆₀Ga₂₋₉, où les nombres sont des pourcentages atomiques d'éléments respectifs ; ou
la phase nanocristalline riche en Cu est constituée de Fe₁₀₋₁₅RE₃₀₋₅₀Cu₃₀₋₄₄Ga₇₋₁₀; où les nombres sont des pourcentages atomiques d'éléments respectifs ; ou
la phase nanocristalline riche en Cu est constituée de Fe₇RE₃₉Cu₄₅Ga₉, Fe₁₂RE₂₆Cu₅₈Ga₄, Fe₁₄RE₃₂Cu₅₂Ga₂, Fe₁₀RE₅₀Cu₃₃Ga₇, Fe₁₃RE₃₈Cu₄₂Ga₇, Fe₁₄RE₃₄Cu₄₂Ga₁₀ ou F₁₅RE₄₄Cu₃₁Ga₁₀, où les nombres sont des pourcentages atomiques d'éléments respectifs.

3. Matériau d'aimant néodyme-fer-bore selon la revendication 1, **caractérisé en ce que** le pourcentage en volume de la phase nanocristalline riche en Cu dans la zone triangulaire intergranulaire est de 4 à 9 %, de préférence de 4,5 %, 4,2 %, 6,1 %, 6,6 %, 7,5 %, 7,8 % ou 8,5 %.

4. Matériau d'aimant néodyme-fer-bore selon la revendication 1, **caractérisé en ce que** :
le matériau d'aimant néodyme-fer-bore comprend les constituants suivants en % en masse de Nd : 24,75 %, Pr : 8,25 %, Al : 1,00 %, Cu : 0,25 %, Ga : 0,12 %, Co : 0,80 %, Nb : 0,15 %, B : 0,98 % et Fe : 63,7 % ; ou
le matériau d'aimant néodyme-fer-bore comprend les constituants suivants en % en masse de Nd : 24,00 %, Pr : 8,00 %, Al : 0,80 %, Cu : 0,35 %, Ga : 0,16 %, Co : 0,50 %, Zr : 0,10 %, Ti : 0,10 %, B : 0,98 % et Fe : 65,01 % ; ou
le matériau d'aimant néodyme-fer-bore comprend les constituants suivants en % en masse de Nd : 23,25 %, Pr : 7,75 %, Al : 0,50 %, Cu : 0,50 %, Ga : 0,18 %, Co : 1,00 %, Nb : 0,20 %, B : 0,96 % et Fe : 65,66 % ; ou
le matériau d'aimant néodyme-fer-bore comprend les constituants suivants en % en masse de Nd : 30,00 %, Dy : 0,20 %, Al : 0,30 %, Cu : 0,50 %, Ga : 0,10 %, Co : 0,50 %, Nb : 0,18 %, B : 0,95 % et Fe : 67,27 % ; ou
le matériau d'aimant néodyme-fer-bore comprend les constituants suivants en % en masse de Nd : 30,00 %, Dy : 0,20 %, Al : 0,30 %, Cu : 0,60 %, Ga : 0,10 %, Co : 0,50 %, Nb : 0,18 %, B : 0,95 % et Fe : 67,17 % ; ou
le matériau d'aimant néodyme-fer-bore comprend les constituants suivants en % en masse de Nd : 30,00 %, Dy : 0,20 %, Al : 0,30 %, Cu : 0,50 %, Ga : 0,05 %, Co : 0,50 %, Nb : 0,18 %, B : 0,95 % et Fe : 67,32 % ; ou
le matériau d'aimant néodyme-fer-bore comprend les constituants suivants en % en masse de Nd : 30,00 %, Dy : 0,20 %, Al : 0,30 %, Cu : 0,75 %, Ga : 0,05 %, Co : 0,50 %, Nb : 0,18 %, B : 0,95 % et Fe : 67,07 %.

5. Procédé de préparation pour un matériau d'aimant néodyme-fer-bore **caractérisé par le fait qu'**il comprend les étapes suivantes de préparation d'une ébauche d'aimant à partir des constituants respectifs du matériau d'aimant néodyme-fer-bore selon l'une quelconque des revendications 1 à 4 ; et de soumission de l'ébauche d'aimant à un traitement de vieillissement pour obtenir le matériau d'aimant néodyme-fer-bore, dans lequel le traitement de vieillissement comprend un vieillissement primaire et un vieillissement secondaire, et le vieillissement secondaire est réalisé à une température de 440 à 480 °C ;
dans lequel le vieillissement primaire est réalisé à une température de préférence de 800 à 1200 °C, plus préférentiellement de 900 °C ;
le vieillissement primaire est réalisé pendant une durée de 2 à 4 h, plus préférentiellement de 3 h ;
de préférence, lorsque le vieillissement primaire est achevé, l'ébauche d'aimant est refroidie jusqu'à température ambiante et soumise ensuite au vieillissement secondaire ;
le traitement de vieillissement secondaire est réalisé à une température de préférence de 440 °C, 450 °C, 460 °C ou 480 °C ;
le traitement de vieillissement secondaire est réalisé pendant une durée de préférence de 2 à 4 h, plus préférentiellement de 3 h ;
le procédé de préparation pour l'ébauche d'aimant comprend de préférence la soumission des constituants respectifs pour le matériau d'aimant néodyme-fer-bore à une fusion, une coulée, une pulvérisation, un façonnage et un frittage tour à tour ;
la fusion est réalisée à une température de préférence de 1550 °C ou moins, plus préférentiellement de 1480 à 1550 °C, et encore plus préférentiellement de 1520 °C ;
la fusion est de préférence effectuée dans un environnement sous vide ;
la fusion est de préférence effectuée selon un procédé de coulée à solidification rapide ;
la fusion est réalisée à une température de préférence de 1390 à 1460 °C, plus préférentiellement de 1410 °C ;
la pulvérisation comprend de préférence une pulvérisation de décrépitation par hydrogène et une pulvérisation de broyeur à jet tour à tour ; la pulvérisation de décrépitation par hydrogène comprend de préférence des traitements d'absorption d'hydrogène, de déshydrogénation et de refroidissement ; l'absorption d'hydrogène est réalisée à une pression d'hydrogène de préférence de 0,05 à 0,12 MPa, plus préférentiellement de 0,085 MPa ; la déshydrogénation comprend de préférence un chauffage jusqu'à 300 à 600 °C dans un état sous vide ; la pulvérisation de broyeur à jet est de préférence effectuée dans une atmosphère ayant une teneur en gaz oxydant n'excédant pas 100 ppm ; la pulvérisation de broyeur à jet est réalisée dans une chambre de broyage ayant une pression de préférence de 0,5 à 1 MPa, plus préférentiellement de 0,7 MPa ; l'ébauche d'aimant obtenue après la pulvérisation de broyeur à jet possède une taille particulaire D50 de préférence de 3 à 6 µm, plus préférentiellement de 4,2 µm ;
le façonnage est de préférence un façonnage par champ magnétique ; le façonnage par champ magnétique est de préférence effectué sous une intensité de champ magnétique de 1,8 à 2,5 T ; le façonnage par champ magnétique est de préférence effectué dans une atmosphère protectrice ;
il est préférable d'ajouter un lubrifiant à une poudre obtenue après la pulvérisation avant le façonnage ; le lubrifiant est de préférence le stéarate de zinc ; le lubrifiant possède un pourcentage en masse de préférence de 0,05 à 0,15 %, plus préférentiellement de 0,10 % dans la poudre obtenue après la pulvérisation ; le frittage est de préférence effectué dans un environnement sous vide ; le frittage est réalisé à une température de préférence de 1000 à 1100 °C, plus préférentiellement de 1085 °C ; et le frittage est réalisé pendant une durée de préférence de 4 à 8 heures, plus préférentiellement de 6 heures.

6. Utilisation du matériau d'aimant néodyme-fer-bore selon l'une quelconque des revendications 1 à 4 en tant que composant électronique dans un moteur.
